

## UNITED STATES PATENT OFFICE

RUDOLF BRAUCKMEYER, OF GRUNBERG, GERMANY, ASSIGNOR TO DEUTSCHE WOLLEN-  
WAREN-MANUFAKUR AKTIENGESELLSCHAFT, OF GRUNBERG, SILESIA, GERMANY

## MAKING TONE IN TONE EFFECTS IN WOOLEN FABRICS

No Drawing. Application filed October 25, 1927, Serial No. 228,694, and in Germany October 8, 1927.

This invention relates to a method for producing tone in tone (deux tone) effects in woolen fabrics.

It is known to increase the adsorbability of 5 wool for dyes by treating the wool fiber with certain chemicals and to use this fact for obtaining tone in tone effects in woolen fabrics by treating one part of the undyed wool yarn with cold, diluted sodium hydroxide solution 10 or other strongly alkaline reacting substances, weaving the treated wool yarn together with untreated yarn and dyeing the obtained fabric in one single dye bath with the usual acid wool dyes. The pretreated 15 yarn then adsorbs greater amounts of dye in shorter time, than the untreated yarn, thereby obtaining a good tone in tone effect in the fabric.

This method for producing tone in tone effects has however not found general application, as the pretreatment of the wool with strongly attacking chemicals hurts the wool fibre considerably and even dissolves it partly, thereby changing the physical properties of the wool. Thus for example a wool 20 treated as above described loses at least 40-50% of its strength and extensibility and is therefore not suitable for use.

According to my invention I obtain strongly contrasting tone in tone effects in woolen fabric without hurting the wool fibre to such an extent as above, by pretreating the wool for a short time with solutions of salts, as for example sodium phosphate, sodium borate and the like hydrolytically decomposed, whereby the adsorbability for dyes of the wool fiber is considerably increased. The hydrolytic decomposition referred to in the foregoing sentence results from a double decomposition of 35 the salt and the water into acid ions and hydroxyl ions, the hydroxyl ions being slightly more numerous than the acid ions thus keeping the solution basic to a small degree so as not to injure or dissolve the wool. Compared 40 with the known methods the action of the salts upon the wool fiber is so feeble, that an injury of the wool can scarcely be noticed even by microscopical examination. The 45 change of the wool is so small, that good tone in tone effects are not obtained, when dyeing 50

a fabric made from untreated and pretreated wool with the usual acid wool dyes under the usual dyeing conditions.

I have found that dyes which are seldom or never used for dyeing wool due to their varying affinity for the wool fiber under different conditions of dyeing, i. e., temperature variation, concentration of solution, etc., are well adapted for producing contrasting tone in tone effects in woolen fabric when employed with wool pretreated by my method. Thus 55 for example the diazo and polyazo dyes especially those known in the trade as "Benzo Light" dyestuffs, which are otherwise generally used for dyeing cotton, produce, in a comparatively strongly acid dyeing bath, great 60 differences in color upon untreated and feebly pretreated wool. Whereas these dyes are 65 completely developed only in presence of 6-10% sulfuric acid by a boiling during several hours, a smaller addition of sulfuric acid 70 for example 2% is already sufficient for producing tone in tone effects, as the pretreated wool fiber adsorbs and binds the dye easily.

## Example I

The loose wool or the wool yarn is boiled for about one hour in a bath containing 6% sodium phosphate in order to increase its adsorbability for dyes. The pretreated wool 80 fiber is spun together with untreated wool fiber and then woven or the pretreated wool yarn is woven together with untreated yarn to a fabric having the desired tone in tone design and the obtained fabric is dyed with 85 0.2% Benzo Light red 8 B L color index number 278, 4% acetic acid and 10% Glau- 90 ber's salt. The fabric enters this dyeing bath at temperatures between 35 and 40° C. and the bath is then slowly brought to boil. For the increased dye adsorbability of the pre- 95 treated wool the bath is quickly exhausted, thus only a short boiling period being necessary. It is to be understood that the percentages referred to in this and the following example relate to the weight of the 95 woolen material dyed.

The obtained dyed fabric is especially proof against boiling, which is generally not the case with fabric dyed with the usual acid 100

wool dyes. When tone in tone designs are made according to my invention it is therefore not to be feared that the differences in tone between pretreated and untreated wool are equalized during a longer boiling period.

5 It is further also possible to make use of my invention in those methods, where the dye adsorbability of certain parts of a fabric is increased by printing chemical substances upon the fabric. Until now one has used for this purpose strongly alkaline reacting printing pastes containing for example 450 gr. sodium hydroxide solution of 40° Bé, 125 gr. water, 75 gr. glycerine, 250 10 gr. tragacanth (65:1000) and 100 gr. British gum. These pastes are however real solvents for the wool and have therefore not been used, as they injure the wool fibre considerably.

15 20 However when using the above mentioned dye groups one obtains, by printing the fabric with a paste containing for example 150 gr. sodium borate and 850 gr. tragacanth solution and steaming the printed texture 25 for a short time, such an increased dye adsorbability of the printed parts, without injuring the wool fibers, that wonderful tone in tone effects are obtained with a single dye bath.

30 *Example II*

The fabric is printed with a paste containing 150 parts sodium borate and 850 parts tragacanth solution, then steamed during 10 to 15 minutes, rinsed and dyed in a bath containing 0.5% polyazo dyestuff and 2% sulfuric acid and having a temperature of 30° C. at the start.

I claim:

40 1. A method for producing tone in tone effects in woolen fabrics comprising the steps of treating those parts of the fabric, which are to have the deeper tone, with solutions of hydrolytically decomposed salts and dyeing the fabric with azo dyes having according 45 to the dyeing conditions a varying affinity for the wool fibre.

50 55 2. A method for producing tone in tone effects in woolen fabrics comprising the steps of treating those parts of the fabric, which are to have the deeper tone, with solutions of hydrolytically decomposed salts and dyeing the fabric with dyes containing at least two azo groups and having according to the dyeing conditions a varying affinity for the wool fibre.

In testimony whereof I affix my signature.  
RUDOLF BRAUCKMEYER.